

## UNITED STATES PATENT OFFICE.

EUGEN STRASSER, OF RORSCHACH, SWITZERLAND, ASSIGNOR TO MAX DIETIKER, OF ZURICH, SWITZERLAND.

PROCESS FOR THE PRODUCTION OF ALUMINUM CASTINGS AND MOLDS FOR USE THEREIN.

No Drawing. Application filed December 7, 1925, Serial No. 73,865, and in Germany December 13, 1924.

This invention relates to the production of aluminum castings, which term includes castings of aluminum alloys, for example aluminum-zinc castings, and to molds for use 5 therein.

The object of the invention is to enable chilled aluminum castings to be produced having high grade mechanical and physical properties.

10 According to the invention the mold in which the aluminum casting is to be effected is made of a mixture of molding sand and metal or metallic or metalliferous compounds, in a divided form for instance in a granular, pul-

15 verulent or powdered form.

The mixture is preferably effected while the sand is in a loose state and so that the metal, or metallic, or metalliferous material is uniformly distributed throughout the sand.

20 When an aluminum casting is made in a mold of this nature the resulting casting has high grade mechanical and physical properties. Particularly good results are obtained with alloys of aluminum and zinc, or zinc and 25 other and more difficultly fusible metals.

When an aluminum zinc alloy such, for example, as the so-called German alloy is used as the metal to be cast a most surprising result is obtained. This alloy, which contains 10% 30 of zinc, 2% of copper and 88% of aluminum and hitherto having comparatively low grade qualities, shows a marked improvement, its properties considerably surpassing for instance those of pure aluminum, that is castings of this hitherto low grade alloy can be produced exhibiting mechanical properties which are far above those of all aluminum alloys hitherto regarded as high grade. The 35 product of the process according to the invention is principally intended to rank as a

40 specifically lighter substitute for cast iron, particularly grey cast iron and is distinguished mainly by its high resistance to fracture, its limit of elasticity, Brinell hardness and the ease with which it can be worked with cutting tools like a good brass.

45 Further advantages to be obtained are the

ease with which the mold can be produced and in the uniform composition throughout the whole of the mold which is necessary for the 50 final product.

The better result may depend inter alia on the better permeability of the mold and the possibility thus afforded of the mold taking up and carrying off more moisture, both during and after the casting operation, but particularly that a more uniform cooling action is obtained.

The best results as regards mechanical properties become manifest after a period of 60 about fourteen days, after casting.

Examples of ores or metalliferous materials which give good results are chalcocite (copper glance)  $Cu_2S$ , or chalcopyrites (copper pyrites)  $CuFeS_2$ .

These materials are roasted, and in the roasting process, crumble to a fine powder which is highly suitable for the purpose.

Copper powder or filings may also be used effectively.

The proportions of molding sand and additive employed to form the molding mixture vary according to the nature of the casting to be produced, for example in the production of castings having a thickness of wall of say 10 to 15 millimetres, a mixture composed of 75% molding sand and 25% additive will be found satisfactory, whereas for castings having a thickness of wall of 15 to 30 millimetres, a molding mixture composed of 50% molding sand and 50% additive is more suitable, while for castings having a thickness of wall of 30 to 45 millimetres the molding mixture may be composed of 25% molding sand and 75% additive.

It is unnecessary to subject material obtained by the present process to hot or cold treatment for ageing purposes, as is necessary in the case of duralumin for example, and it is found that the damper the molding composition the greater is the ageing effect. The addition of zinc to the metal to be cast should not exceed 18%.

I claim:—

1. A process for the production of chilled aluminum castings which consists in casting the molten aluminous material in a mold composed of a mixture of molding sand and 5 roasted copper ore in a finely divided state, for the purpose hereinbefore set forth.

2. A mold, for use in the casting of aluminum castings, composed of a mixture of molding sand and copper ore in a finely divided

state, substantially as and for the purpose 10 hereinbefore set forth.

3. A mold, for use in the casting of aluminum castings, composed of molding sand and finely divided chalcocite, substantially as and for the purpose hereinbefore set forth.

In testimony whereof I affix my signature.

EUGEN STRASSER.